

# UNITED STATES PATENT OFFICE.

OTTO RÖHM, OF DARMSTADT, GERMANY.

## PROCESS FOR MAKING LEATHER WITH THE ASSISTANCE OF IRON SALTS.

1,364,316.

Specification of Letters Patent.

Patented Jan. 4, 1921.

No Drawing. Application filed March 10, 1917, Serial No. 154,033. Renewed May 28, 1920. Serial No. 385,064.

*To all whom it may concern:*  
Be it known that I, OTTO RÖHM, a citizen of Germany, residing at No. 4-6 Weiterstädterstrasse, in the city of Darmstadt, Grand Duchy of Hessa, German Empire, have invented Improvements in Processes for Making Leather with the Assistance of Iron Salts; and I do hereby declare that the following is a full, clear, and exact description 10 of the same.

It is well known that skins can be tanned with the assistance of ferric iron oxid salts. Heretofore however certain difficulties arose which prevented the production of a practically useful iron leather. If the salts are too acid the depilated skins are indeed tanned throughout, but the leather is not stable in light and becomes brittle and grain-broken. If basic salts are used, only the outer layers 15 are tanned, while the inner layers are slack tanned, and in this case also the grain breaks.

Now it has been found that with ferric iron oxid salts leather can be made which is stable in water and light and does not 20 become cracked in grain, if previous, or in addition, to the tanning with iron salts, a tanning process is carried out with aldehydes, for example formaldehyde. The iron salts can be more or less basic or acid, and 25 the leather produced, like alum leather, can be dried acid, or like chrome leather, it can be neutralized, before being dried.

The aldehyde tanning moreover renders it possible to incorporate any desired quantity of iron oxid, up to 30% and more, in the skin, without the leather losing surface, if, alternately, the iron salts are allowed to act and then ammonia, alkalis and alkaline salts are used for neutralizing. In this way 30 leather of different degrees of softness or hardness, even to sole leather, can be produced, and the iron tanned sole leather has, for example, over chrome tanned leather the advantage that in a wet condition it is not 35 slippery, and therefore does not cause the wearer of the boots to fall, like chrome leather.

Example: 100 parts of depilated skins are worked  $\frac{1}{2}$  hour with 200 parts water + 5 parts of 40% formaldehyde solution + 2 parts sodium bicarbonate. The skins are then washed with water and with  $\frac{2}{3}$  basic ferric iron chlorid in doses of 10-20% until the desired quantity of iron has been taken

up. As soon as no more iron is taken up by the depilated skins, they are neutralized with soda.

This iron aldehyde tanning can be combined with a tanning by phenols, naphthols, aromatic carbon acids and vegetable tanning substances, so that a greater variety of leather can be obtained.

By other substances which yield insoluble compounds with iron the properties of this iron leather may also be modified, for example, by soaps, or, with the help of sulfids and polysulfids, sulfur may be incorporated. 65

Further it has been shown that the combination of the iron-aldehyde tanning processes affords a special technical advantage, 70 if, as mentioned in the above example, the process is carried out with basic ferric iron chlorid.

The mineral tanned leather heretofore known and used, which has been made either 75 with aluminium or chrome salts has the property that, in addition to the particular metal oxids, they contain a residue of acids. They are compounds of the skin with basic metal salts. For example, chrome leather 80 contains 3-10% acid, see Jettmar, *Handbuch der Chromgerbung*, 1912, page 115. The consequence of this acid residue is that such leather cannot be well used where it comes into contact with metals, because 85 metals are oxidized.

Now the remarkable fact has been discovered that basic ferric iron chlorid dissociates entirely in the presence of skin and water, the iron combining with the skin, 90 so that a leather is obtained which is entirely free from acid. If however depilated skins impregnated in this way with iron hydroxid are dried they will shrink together and do not yield a technically utilizable leather. The leather is however utilizable, if, according to the present invention, before, or after, the treatment with ferric iron chlorid the skins are tanned with formaldehyde. Sheep skins treated in this 95 way, for example, yield a perfect substitute for chamois leather.

In tanning with basic ferric iron chlorid and aldehyde a neutral iron leather is obtained, which can be used for saddlery and 100 sole purposes, because iron parts do not rust in contact with this leather. If, instead of ferric iron chlorid, ferric iron sulfate for

example, is used, such neutral leather is not obtained.

What I claim and desire to secure by Letters Patent of the United States is:—

- 5 1. The process for producing leather which consists in subjecting the skins to the action of aldehydes and ferric iron salts.
- 10 2. The process for producing leather which consists in subjecting the skins to the action of formaldehyde and ferric iron salts.
- 15 3. The process for producing leather which consists in subjecting the skins to the action of formaldehyde and ferric iron chlorid.
- 20 4. The process for producing leather which consists in subjecting the skins to the simultaneous action of aldehydes and ferric iron salts.
5. The process for producing leather which consists in subjecting the skins to the action of aldehydes and ferric iron salts

and subsequently treating the same with alkalis.

6. The process for producing leather which consists in subjecting the skins to the 25 action of aldehydes and ferric iron salts and neutralizing the same with sodium bicarbonate.

7. The process for producing leather which consists in subjecting the skins to the 30 action of a formaldehyde solution and sodium bicarbonate, then tanning said skins with basic ferric iron chlorid and neutralizing with soda, and then repeating the treatment several times with the ferric iron salt 35 and soda.

8. The process for producing leather which consists in subjecting the skins to the action of aldehyde and ferric iron salts and then to the action of vegetable tanning substances. 40

OTTO RÖHM.